

A. L. D. D'ADRIAN.  
PROCESS OF RECOVERING METALS.  
APPLICATION FILED NOV. 7, 1919.

1,434,485.

Patented Nov. 7, 1922.



## UNITED STATES PATENT OFFICE.

ALEXANDER L. DUVAL D'ADRIAN, OF WASHINGTON, PENNSYLVANIA, ASSIGNOR TO  
B. F. DRAKENFELD & CO. INC., OF NEW YORK, N. Y., A CORPORATION OF NEW YORK.

## PROCESS OF RECOVERING METALS.

Application filed November 7, 1919. Serial No. 336,260.

To all whom it may concern:

Be it known that I, ALEXANDER L. DUVAL D'ADRIAN, a citizen of the Republic of France, and a resident of Washington, county of Washington, and State of Pennsylvania, have invented certain new and useful Improvements in Processes of Recovering Metals, of which the following is a specification.

10 Heretofore in the production of the oxides or salts of chromium, zirconium, vanadium, uranium, cobalt, silver, or nickel from their ores, disadvantages have been encountered in obtaining the oxides or salts, free from 15 the iron that may be present in the ores, or in the residues, or free from other impurities, or in the separation of one or more metallic compounds from a group.

The object of my invention is to provide 20 a process by means of which the oxides or salts such as chlorides, of chromium, zirconium, vanadium, uranium, cobalt, silver, or nickel, may be readily obtained from their respective ores or from residues containing 25 chromium, zirconium, vanadium, uranium, cobalt, silver, or nickel, by means that are simple and efficient and commercially practicable.

In order to carry out my invention, I 30 will describe the same in the light of one embodiment, and more particularly refer by way of example, to the treatment of chromium ore, and the obtaining of chromium oxide from the ore, with the understanding, 35 however, that parts of this process may be applied to the treatment of zirconium, vanadium, uranium, cobalt, silver or nickel, with, however, certain modifications which will hereinafter appear.

40 In carrying out my process, for the purpose of obtaining chromium oxide practically free from iron or other impurities, I take the chromium ore as it comes from the mines, and grind it very finely into powdered form. 45 This chromium ore is usually called chromite. The object of grinding the ore into finely powdered form, is to get as large a surface as possible so that it may be readily treated as hereinafter described. This powdered 50 chromium ore is then mixed with sawdust and with molasses, or with a starch and water mixture, or any other suitable organic compound may be used, adapted to serve as a

binder. The preferable proportions are about as follows, as an example:

55 Chromium ore in 100 parts; sawdust in 15 parts, and the binder in 5 parts.

This mass is then formed into bricks or blocks. These bricks or blocks are then placed in a furnace having a closed muffle, and heated. The heating to which the bricks or blocks are subjected, first carbonizes the sawdust and the binder. Thereby the particles of the chromium ore are separated from each other by spaces filled with gases, 60 and by the carbonized particles, by reason of which the bricks or blocks become of a porous character, and a large surface of exposure of the chromium ore is obtained after the sawdust and binder has been carbonized. Chlorine gas is then injected into the furnace. The chlorine gas penetrates the blocks or bricks and acts on the ore. The chlorine gas is injected through a tube from a suitable storage tank. The muffle during 75 the introduction of the chlorine gas, is brought to a temperature at which the evolution of the iron chloride commences. It is advantageous to maintain the muffle temperature between approximately 450° C. and 80 1000° C., depending upon the ores to be treated.

It is here to be noted that various chromium ores, even from the same mine, require variations in the treatment with respect to the temperatures. The iron of the 85 chromium ore sublimes at about 450° C., though some iron chloride is formed at temperatures below this. It is preferable not to go beyond 1000° C. because chromium chloride sublimes at about 1065° C. The chlorine 90 gas combines with the iron in the chromium ore, and forms iron chloride which passes out of the furnace, flowing through a pipe line. This pipe line may be made transparent by the use of glass or the like, or may 95 be provided with some transparent window so that the contents flowing through the pipe may thereby be visible and may be inspected.

This iron chloride passes through the pipe in the form of a thick vapor of a 100 brown color. The passing of the chlorine gas is continued until no further considerable iron chloride passes through the tube or exhaust pipe which may be readily determined by inspection. In some cases, it is 105 preferable to inject a slight amount of steam

either into the muffle by means of a separate tube, or through the same tube with the chlorine gas. This steam acts to form a certain amount of chloride of iron containing six 5 molecules of water ( $\text{FeCl}_3 \cdot 6(\text{H}_2\text{O})$ ), which very readily volatilizes, namely at a temperature of about  $280^\circ$  to  $285^\circ$  C. The injection of the chlorine gas is continued until the brown vapor practically ceases, whereupon it 10 is shut off. It may be mentioned that when the brown vapor stops, practically all the iron of the ore has been combined with the chlorine gas, and carried off in the form of iron chloride. This may be conducted to cooling 15 vessels whereby it may be condensed into a marketable article, by the utilization of temperatures below about  $450^\circ$  C.

The heating operation is continued for about fifteen minutes or more, to assist in 20 driving off any iron chloride which may be in the muffle, and air is passed through the muffle to eliminate as much as possible any chlorine gas present in the muffle. It is preferable to use moist air. The air also brings 25 about the combustion of the carbon particles. The remaining content of the muffle is composed of chromium oxide with some chrome chloride, and small amounts of silica or other impurities, but practically free from iron. 30 After the chrome oxide has thus been obtained practically free from iron, the chromium oxide and any chromium chloride remaining in the furnace are taken out of the furnace and the chromium oxide is freed 35 from the chromium chloride by dissolving out the chromium chloride in a manner well known to the art.

For commercial purposes, it is preferable to use a rotary muffle kiln or muffle furnace. 40 In the use of a rotary furnace, no molding of the ore is necessary. This is due to the agitation to which the ground ore is subjected by the rotation of the furnace and the consequent production of new surfaces of contact 45 of the particles of the ore with the gas in the muffle. In the use of a rotary furnace, the ore in finely powdered form is mixed with carbon and then heated and subjected to the action of the chlorine gas for the elimination 50 of the iron from the ore. It is not always necessary to use the carbon. It has been found that with the use of carbon, lower temperatures may be utilized as the presence of carbon facilities and makes more 55 rapid the action of the gas. The treatment of the contents of the muffle is carried out as above described. The remaining chromium oxide with chromium chloride such as remains in the furnace, is treated as above 60 described, namely by dissolving out the chromium chloride in a manner well known to the art. Whatever silica remains here, as also in the furnace before mentioned, may be removed by processes well known in the art, 65 as for example, by hydrofluoric acid.

The process as above described, is based upon the regulation of the temperatures during the passage of the chlorine gas through the furnace and its coming into contact with the ore, it being important to so regulate the temperatures that only a selective volatilization and subliming will take place, that is, such temperatures as will cause the iron to combine with the chlorine gas to form iron chlorides and will practically sublime or 70 distill only the iron chlorides. In other words, fractional sublimation or distillation is obtained.

If desired, this selective temperature method may be replaced by another method 80 which utilizes temperatures higher than  $1000^\circ$  C. or  $1065^\circ$  C. at which latter temperature chromium chloride is formed and sublimes, and which carries out the process until 85 all of the materials in the furnace are volatilized and sublimed in the form of chlorides. In this process, temperatures are utilized from  $450^\circ$  C. upwards.

In the accompanying drawing I have disclosed a typical apparatus by means of which 90 the present process may be successfully practiced. In this drawing 5 designates the rotary muffle kiln or furnace having an outer wall or shell 6 of refractory material. To one end of the rotary kiln a chlorine gas 95 storage tank 7 is connected through the medium of the pipe 8, which is coupled to a pipe 9 for supplying air under pressure, and to a steam supply pipe 10. A suitable gas tight fitting or connection is provided between the gas supply pipe and the end of the rotary kiln. A series of condensers 12 are connected in series to each other, each condenser being arranged in conjunction with a heating chamber 13. The first condenser 105 in the series is connected by a gas tight fitting 14 to the other end of the rotary kiln, while the last condenser in the series is connected by a pipe 15 with a pump 16, which creates a partial vacuum in the several condensers and draws the chlorine gas entering 110 the condensers from the furnace through the said pipe 15, and returns the same to the storage tank 7 through the pipe connection 17 between said tank and the pump 16. It 115 will be understood that the drawing is simply illustrative of one possible construction of apparatus which may be employed in the practice of my improved process on a commercial basis.

It will be readily appreciated that various other alternative constructions might be employed. Thus, as hereinafter noted, instead of providing the single condenser 12, a plurality of groups of condenser units may be 125 utilized, and such groups of units connected in series with each other whereby a succession of condensations will occur in each condenser group.

Above the temperature of  $1065^\circ$  C. the 130

chromium oxide is transferred into a chloride and is sublimed at or above this temperature, and practically all the rest of the materials are transferred into chlorides and 5 are volatilized and sublimed. During the time that the ore is subjected to the temperatures ranging from the initial temperature of 450° C. and then through the various temperatures up to 1065° C. and above 10 1065° C. the vapors or sublimes are conducted from the furnace into condensers. These condensers are arranged in series, that is, the first condenser is in communication with the furnace and thereafter each following condenser communicates with the one preceding. These condensers are maintained at different temperatures. The first condenser, or in case more than one is desired to be used, then the first condenser or the 15 first group is maintained at one constant temperature, and this temperature is higher than any of the other temperatures in any of the other condensers. The temperature of the first condenser or group of condensers 20 is selected to bring about the deposit of chromium chloride. If chromium chloride is maintained at a temperature less than 1065° C., it will deposit. For this reason the first condenser or the first group of condensers which has for its object to bring 25 about the deposit of the chromium chloride, are maintained at a temperature between 460° to 500° C. All substances which maintain their subliming at temperatures below 30 500° C. will flow from the first group of condensers to the next or number two group. This number two group of condensers is maintained at a temperature below 450° C. but above 220° C. It is within this range of 35 temperatures that iron chloride deposits in the form of  $FeCl_3$ . The other substances which keep on subliming, pass off or continue into the number three group of condensers. This third group of condensers is 40 maintained at a temperature below 57° C. and above 40° C. This range of temperatures brings about the deposit of various silicon chlorides, as per example,  $SiCl_3$  below 145° C.,  $SiCl_4$  below 57° C., and  $Si_3Cl_8$  45 below 210° C. Certain substances, as for instance  $FeCl_3 \cdot 6(H_2O)$  are carried off from these condensers into a next group, and this last group is kept at temperatures below 37° C., whereupon the  $FeCl_3 \cdot 6(H_2O)$  50 deposit.

I have spoken of groups of condensers for each step, but it is clear that in some cases, one condenser may take the place of a group. The advantage, however, of more than one 55 condenser for each step is that in the first condenser of a group, for instance at the step wherein it is desired to deposit chromium chloride, perhaps not the entire quantity of chromium chloride will deposit, and 60 part of the chromium chloride will be car-

ried off with the remaining chlorides, and deposited in a subsequent unit of the same group. Similarly, in the second step where iron chloride is deposited, parts of the iron chloride may pass off from the first condenser of this group and will deposit in a subsequent unit of the same group. Similarly, in the subsequent steps it is preferable to use two or more condensers. 70

It will therefore be seen that by the various groups of condensers regulated at temperatures which control the condensation and deposit, all the various chlorides which have passed out of the furnace will be individually isolated. 75

The chromium chloride deposited in the first condenser or a group of condensers, is then treated in a manner well known to the art to secure chromium or its compounds, as for instance chromium oxide. Similarly, the other chlorides may be utilized. Such portions of chlorine gas as comes from the muffle and pass through the condensers, may be collected and recovered. 80

In carrying out the process, it must be remembered that ores from the same mine are different in their characteristics and that it has been found desirable to select portions of the ore desired to be treated and subject them to a preliminary test to ascertain their characteristics. When this preliminary test has been completed and the characteristics of the ore have been ascertained, then one of the above two methods of treatment may be employed as above described. Some ores 90 will be better treated with a selective volatilization, others with a complete volatilization and a selective condensation. 95

I have referred to the use of chromium ore, but it is clear that other ores may be 100 treated in a similar manner.

In regard to vanadium and uranium, it has been found that the complete volatilization and selective condensation method is usually more advantageous. 110

Vanadium ores may contain vanadium, in addition to uranium, lead, silica, iron, barium and other constituents, and by selective condensation vanadium, uranium, silica and iron can be separated. In the case of zirconium 115 ores which may contain silica, iron and titanium, the zirconium, titanium, silicon and iron can be similarly separated. In case of cobalt ores, which, in addition to cobalt, usually contain nickel, silver, iron, arsenic, 120 antimony and silicon, these may be all selectively condensed, or the cobalt ore may be first roasted to remove arsenic and antimony, and then the cobalt, nickel, silver, iron and silicon, selectively condensed. I have spoken 125 of ores, but it is clear that residues may be similarly treated.

In the case of a cobalt ore or a residue containing cobalt, it is necessary in carrying out the above described methods, to remem- 130

ber and be guided thereby, that cobalt chloride sublimes at temperatures about 700° C. Silver chloride sublimes at temperatures about 800° to 900° C. and nickel chloride 5 sublimes at temperatures about 600° to 700° C. Arsenic and antimony is usually generated by roasting and arsenic chloride distills at temperatures below about 130° C. The different antimony chlorides distill at various 10 temperatures above about 102° C., and below about 225° C. The iron chloride as heretofore, sublimes at about 450° C. and the  $\text{FeCl}_3 \cdot 6(\text{H}_2\text{O})$  distills at below about 37° C. The silica chlorides distill at temperatures as 15 follows:

$\text{SiCl}_3$  below about 145° C.,  
 $\text{SiCl}_4$  below about 87° C.,  
 $\text{Si}_2\text{Cl}_5$  below about 210° C.

In the case of vanadium ores or residues, 20 the several vanadium chlorides, distill at below at above about 126.5° C., and below 154° C. Uranium chloride distills below about 750° C. The iron chloride and  $\text{FeCl}_3 \cdot 6(\text{H}_2\text{O})$  distill as heretofore stated. Silica 25 chlorides distilled as heretofore stated. The lead chloride sublimes at about 861° to 954° C. and the barium chloride is left as an acid.

In the case of zirconium ores or residues, 30 titanium chloride distills at below about 136 $\frac{1}{2}$ ° C. The silicon chlorides and iron chlorides as heretofore, and the zirconium chloride at 400° C.

Among the ore residues that I have treated 35 is speiss. I have also treated metal alloys for the separation of the metals composing the same. I believe my methods are also applicable to the treatment of slags and mattes.

I have described the above as embodiments 40 of my invention but it is clear that changes may be made therein without departing from the spirit and scope of the invention as defined in the appended claims.

I claim:

45 1. The process of obtaining chromium, zirconium, vanadium, uranium, cobalt, silver, or nickel in the form of oxides or chlorides or other chlorine compounds from their respective ores, or from residues containing 50 chromium, zirconium, vanadium, uranium, cobalt, silver, or nickel, which consists in subjecting an ore or residue to a heat treatment in the presence of chlorine gas, for combining the iron of the ore or residue with the 55 chlorine gas, and then removing the iron chloride from the ore or residue.

2. The process of obtaining chromium, zirconium, vanadium, uranium, cobalt, silver, or nickel in the form of oxides or chlorides 60 or other chlorine compounds from their respective ores, or from residues containing chromium, zirconium, vanadium, uranium, cobalt, silver or nickel, which consists in subjecting an ore or residue to a heat treatment 65 in the presence of moist chlorine gas, for

combining the iron of the ore or residue with the chlorine gas, and then removing the iron chloride from the ore or residue.

3. The process of obtaining chromium, zirconium, vanadium, uranium, cobalt, silver, 70 or nickel in the form of oxides or chlorides or other chlorine compounds from their respective ores, or from residues containing chromium, zirconium, vanadium, uranium, cobalt, silver, or nickel, which consists in 75 subjecting an ore or residue and carbon mixed therewith to heat treatment in the presence of chlorine gas for combining the iron of the ore or residue with the chlorine gas, and then removing the iron chloride 80 from the ore or residue.

4. The process of obtaining chromium, zirconium, vanadium, uranium, cobalt, silver, or nickel in the form of oxides or chlorides or other chlorine compounds from their 85 respective ores, or from residues containing chromium, zirconium, vanadium, uranium, cobalt, silver, or nickel, which consists in heating an ore or residue in the presence of carbon, then subjecting the ore or residue 90 and carbon to further heat treatment at a relatively higher temperature and to the simultaneous action of chlorine gas, to thereby form a chloride and then removing the chloride.

5. The step in the art, which consists in removing the iron from chromium, zirconium, vanadium, uranium, cobalt, silver, or nickel ores or residues, containing chromium, zirconium, vanadium, uranium, cobalt, silver, or nickel, by combining the iron of the ore or residue with chlorine gas under the action of heat to form iron chlorides.

6. The step in the art which consists in converting the constituents of chromium, 105 zirconium, vanadium, uranium, cobalt, silver, or nickel ores or residues containing chromium, zirconium, vanadium, uranium, cobalt, silver, or nickel, to chlorides, by combining the metals of the ore or residue with 110 chlorine gas under the action of heat.

7. The process of recovering chromium and iron from ores or residues containing the same and separating them from each other, comprising finely grinding the ore 115 or residue to obtain a large reaction-surface, mixing the same with an easily carbonizable filler and binder, briquetting the mixture, heating the same to carbonize the filler and binder to produce a highly porous texture, 120 whereby the subsequent action of chlorine gas on the metal-content of the mixture is facilitated, subjecting the latter to the action of chlorine gas at a temperature sufficient to distill the iron chlorides but not 125 chromium chloride, condensing the iron chlorides and treating the remaining reaction-mass to recover the chromium contents.

8. The process of recovering chromium and iron from ores or residues containing 130

- the same and separating them from each other, comprising finely grinding the ore or residue to obtain a large reaction-surface, mixing the same with sawdust and a binder, 5 briquetting the mixture, heating the same to carbonize the filler and binder to produce a highly porous texture, whereby the subsequent action of chlorine gas on the metal-content of the mixture is facilitated, subjecting the latter to the action of chlorine 10 gas at a temperature sufficient to distill the iron chlorides but not chromium chloride, condensing the iron chlorides and treating the remaining reaction-mass to recover the 15 chromium contents.
9. The process of recovering chromium and iron from ores or residues containing the same and separating them from each other, comprising finely grinding the ore or residue to obtain a large reaction-surface, 20 mixing the same with an easily carbonizable filler and binder, briquetting the mixture, heating the same to carbonize the filler and binder to produce a highly porous texture, 25 whereby the subsequent action of chlorine gas on the metal-content of the mixture is
- facilitated, subjecting the latter in the presence of steam to the action of chlorine gas at a temperature sufficient to distill the iron chlorides but not chromium chloride, condensing the iron chlorides and treating the remaining reaction-mass to recover the 30 chromium contents.
10. The process of obtaining chromium, zirconium, vanadium, uranium, cobalt, silver, or nickel in the form of oxides or chlorides or other chlorine compounds from their respective ores, or from residues containing chromium, zirconium, vanadium, uranium, cobalt, silver, or nickel, which consists in 35 subjecting an ore or residue to a heat treatment in the presence of chlorine gas, for combining the iron of the ore or residue with the chlorine gas, and then removing the iron chloride from the ore or residue, so 40 as to leave the other metallic constituents as oxides or salts.

In testimony that I claim the foregoing as my invention, I have signed my name hereunder.

ALEXANDER L. DUVAL D'ADRIAN.